

Feb. 28, 1967

J. B. GERO

3,305,901

VACUUM CASTING METHOD OF MULTIPLE INGOT CASTING

Filed June 12, 1963

12 Sheets-Sheet 1

*Fig. 1.*



*Fig. 2.*



*Inventor:*  
*John B. Gero,*  
*by* *Manus H. Hamilton*  
*Attorney*

Feb. 28, 1967

J. B. GERO

3,305,901

VACUUM CASTING METHOD OF MULTIPLE INGOT CASTING

Filed June 12, 1963

12 Sheets-Sheet 2

Fig. 3.



Inventor:

John B. Gero,  
2029

Miner & Hamilton

Attorney

Feb. 28, 1967

J. B. GERO

3,305,901

VACUUM CASTING METHOD OF MULTIPLE INGOT CASTING

Filed June 12, 1963

12 Sheets-Sheet 3

Fig. 4.



Fig. 5.



Fig. 6.



Inventor:  
John B. Gero,  
by *James A. Hamilton*  
Attorney

Feb. 28, 1967

J. B. GERO

3,305,901

VACUUM CASTING METHOD OF MULTIPLE INGOT CASTING

Filed June 12, 1963

12 Sheets-Sheet 4



*Inventor:*  
R. J. John B. Gero,  
by Maurice H. Hamilton  
*Attorney*

Feb. 28, 1967

J. B. GERO

3,305,901

VACUUM CASTING METHOD OF MULTIPLE INGOT CASTING

Filed June 12, 1963

12 Sheets-Sheet 5

*Fig. 9.*



*Fig. 8.*



*Inventor:*  
*John B. Gero,*  
*by* *Marion H. Hamill,*  
*Attorney*

Feb. 28, 1967

J. B. GERO

3,305,901

VACUUM CASTING METHOD OF MULTIPLE INGOT CASTING

Filed June 12, 1963

12 Sheets-Sheet 6

*Fig. 10.*



*Fig. 10a.*



*Fig. 10b.*



*Fig. 10c.*



*Inventor:*  
*John B. Gero,*  
*By: Munro H. Hamilton*  
*Attorney*

Feb. 28, 1967

J. B. GERO

3,305,901

VACUUM CASTING METHOD OF MULTIPLE INGOT CASTING

Filed June 12, 1963

12 Sheets-Sheet 7

*Fig. 11.*



*Inventor:*  
*John B. Gero,*  
*by* *Mauris B. Hamilton*  
*Attorney*

Feb. 28, 1967

J. B. GERO

3,305,901

VACUUM CASTING METHOD OF MULTIPLE INGOT CASTING

Filed June 12, 1963

12 Sheets-Sheet 8

*Fig. 12.*



Inventor:  
John B. Gero,  
By: Max H. Hamilton  
Attorney

Feb. 28, 1967

J. B. GERO

3,305,901

## VACUUM CASTING METHOD OF MULTIPLE INGOT CASTING

Filed June 12, 1963

12 Sheets-Sheet 9



Inventor:  
John B. Geo,  
by Munro H. Hamilton  
Attorney

Feb. 28, 1967

J. B. GERO

3,305,901

VACUUM CASTING METHOD OF MULTIPLE INGOT CASTING

Filed June 12, 1963

12 Sheets-Sheet 10



Inventor:  
John B. Gero,  
by Munro V. Hamilton  
Attorney

Feb. 28, 1967

J. B. GERO

3,305,901

VACUUM CASTING METHOD OF MULTIPLE INGOT CASTING

Filed June 12, 1963

12 Sheets-Sheet 11



Inventor:  
John B. Gero,  
by Munro & Hamilton  
Attorney

Feb. 28, 1967

J. B. GERO

3,305,901

VACUUM CASTING METHOD OF MULTIPLE INGOT CASTING

Filed June 12, 1963

12 Sheets-Sheet 12



Inventor:  
John B. Gero,  
by *James A. Hamilton*  
*Attorney*

1

3,305,901

## VACUUM CASTING METHOD OF MULTIPLE INGOT CASTING

John B. Gero, Manchester-by-the-Sea, Mass., assignor to  
Gero Metallurgical Corporation, Boston, Mass., a cor-  
poration of Delaware

Filed June 12, 1963, Ser. No. 287,416

2 Claims. (Cl. 22—209)

The present application is a continuation-in-part of application Serial No. 122,440 filed July 7, 1961, now abandoned, and application Serial No. 235,953 filed November 7, 1962, now Patent No. 3,182,359 dated May 11, 1965.

This invention relates to methods and apparatus for vacuum casting of molten metals and, especially to vacuum casting of heavy forging ingots and the mass production of rolling ingots wherein gaseous components of harmful nature are in part removed from the molten metal during the period that the molten metal is being poured into an ingot mold or ladle.

Removal of gaseous components of harmful nature from molten metal is commonly referred to by the term "degassing." At the present time degassing is conventionally carried out by several different methods, including the "stream droplet" method and the "lift" or "recirculating" method. The present invention and the co-pending applications referred to are in general concerned with novel methods and apparatus for carrying out degassing by the stream droplet technique utilizing a casting mold and a degassing chamber which is required to be secured to the casting mold in tightly sealed relationship for casting under a high vacuum.

In conventional apparatus heretofore used in the stream droplet technique, problems are encountered in maintaining a satisfactory high vacuum. To evacuate gases rapidly from the mold and the degassing chamber to a satisfactory degree requires extremely efficient sealing means and large volume pumping equipment. Since the vacuum must be fully maintained throughout the metal pouring interval there is a period during which the sealing means may be exposed to temperatures which will affect the sealing means. Moreover, there arises a problem of dimensional instability on the part of those surfaces which support the sealing means. This dimensional instability is produced by thermal shock from hot molten metal flowing into the mold and causing differential expansion of parts. A still further consideration is seal replacement where successive ingots are being poured continuously in the steel foundry. This type of continuous operation may require pouring equipment of a construction such that it may be quickly assembled and sealed on any one of a series of relatively rough surfaced, non-uniform casting molds to facilitate production of either large forging ingots or small rolling ingots as may be required from time to time. Existing equipment, so far as I am aware, does not meet these requirements. The methods and apparatus presently employed are unsatisfactory in maintaining a seal which will provide for holding a suitable vacuum and do not provide any practical means of seal replacement.

It is a chief object of the invention to improve methods and apparatus for vacuum casting and to devise means for more effectively and quickly establishing and maintaining a degassing chamber vacuum in order to produce quality steels with desirable magnaflux and micro-cleanliness ratings and to make possible vacuum casting of multiple large or small ingots from one heat or ladle. In such objectives the provision of a vacuum casting system of relatively small volume and more efficient pumping characteristics is of importance.

Another object of the invention is to devise a new combination of sealing compound and casting apparatus for

2

vacuum casting whereby unusual sealing effects may be accomplished and also whereby the evacuation of air to produce a vacuum may be carried out in a highly efficient and rapid manner.

5 A further object of the invention is to devise a method and means for dealing with the problem of dimensional instability and compensating for differential expansion of casting components during the pouring interval.

Still another object is to provide a method of high temperature vacuum sealing which is based on the concept of utilizing a disposable sealing body which is subject to decomposition at relatively high temperatures and which is readily replaced when desired.

10 A further object is to provide improved methods and apparatus for sequence casting of metal ingots into a series of ingot molds in predetermined successive time intervals from a pouring ladle.

15 The method and apparatus of the invention hereinafter disclosed presents several unique techniques for dealing with the problems outlined and realizing the foregoing objectives. These techniques are based on the concept of producing an extremely high vacuum by means of an expansible heat resistant seal, that is a seal sufficiently deformable so as to be expansible with the surfaces to which it is adhered. Nevertheless, the seal is maintained in effect for a relatively short period.

20 In the method of the invention, vacuum casting parts are arranged upon one another and held in sealed relationship for a limited period at least as long as an ingot pouring interval and usually for a little longer than this interval as a factor of safety. The method is further characterized by novel compensation for differential expansion of the components when subjected to thermal shock.

25 In one preferred embodiment the method of the invention includes the steps of evacuating air from a degassing chamber which is mounted on a casting mold; then releasing molten metal from a pouring ladle and conducting the molten metal through the evacuated degassing chamber into a casting mold body whereby a thermally induced differential expansion of the degassing chamber and the casting mold takes place; and simultaneously supporting a yieldable heat resistant sealing body between the degassing chamber and the casting mold, and subjecting the sealing body to forces of deformation to provide a compensating expansion which maintains the sealing body in vacuum tight sealing relationship with both the degassing chamber and the casting mold for a limited period approximately corresponding to the ingot pouring interval.

30 I have discovered that it is possible to start with fluid to wet parts to be sealed, then heat to form deformable solid sealingly adhered to the surfaces it contacts, thereafter to set up on a mold surface an expansible sealing body which although decomposable in the upper range of temperatures induced in a casting mold during an ingot pouring interval, may nevertheless resist thermal attack sufficiently long to yieldably maintain a seal for the period roughly corresponding to the ingot pouring interval.

35 After the pouring interval a rapid increase in the temperature of the casting mold results in "burning off" the sealing body to leave a powdery residue which is readily brushed away and replaced by a new sealing body for the next ingot pouring operation. In thus setting up an expansible sealing body which is to be subjected to forces of deformation, I find that I may also employ means for supporting and reinforcing the sealing body as well as for controlling the degree of differential expansion to which the sealing body may be exposed.

40 As an example of a sealing material which is suitable for this purpose, I may employ a new composition of matter comprising a mixture of three essential components—(I) a low molecular weight glycidyl polyether

(I) a condensation product of a low molecular weight cycidyl polyether and ethylene glycol and; (III) a curing agent composed of pyromellitic dianhydride mixed with anhydride of a dicarboxylic acid. When these components are combined in the hereinafter described proportions a resinous mixture is obtained which upon exposure to moderate heat changes from fluid to solid and thereafter at elevated temperatures resists melting and reappears to a solidified adherent elastic body. In addition to the above ingredients it may be desirable to include various fillers and a cure accelerating agent.

The composition of matter noted above is intended to be representative of sealing compound means which is sufficiently fluid to adhere to metal surfaces of casting members; which is characterized by the ability to cure when brought into contact with metal surfaces heated to temperatures of from room temperature 70° F. to 400° F. to form a tough deformable solid flexible adhesive tenaciously secured to said surfaces; and which in this cured state is capable of resisting flowing or decomposition in the presence of a range of temperatures of from 70° F. to at least 600° F. for a limited period of time corresponding approximately to an ingot pouring interval, and thereafter to be decomposed at elevated temperatures to dry powdery mass which may be readily removed from the mold.

I find that by employing a sealing compound of the class described as an externally located sealing body between the degassing chamber and casting mold, I am enabled to provide for unusually high vacuum as compared with vacuum results obtained with conventional equipment.

As an example of unusually high vacuum, there may be cited absolute pressure readings of an order of magnitude of less than one micron before pouring in the degassing chamber. It should be understood that when pouring starts absolute pressures as defined by micron readings temporarily rise from the one micron reading noted above, to micron readings of as high as 300 to 500 microns, for example. Then, as pouring continues throughout a pouring interval which may range from one minute to ten minutes, the micron reading rapidly decreases, in accordance with the invention, to values well below the 300 to 500 range, for example, down to values from 200 microns all the way to readings as low as 50 microns or even less. In one typical pouring operation carried out in accordance with the method of the invention there has been observed pressures as low as 45 microns. It must be borne in mind that the precise micron value in any given pouring operation, however, depends on the grade of metal which it may be desired to make and other related conditions. This latter micron reading is in contrast to optimum micron readings obtained with conventional equipment of from 700 to 2,000 microns. It should be understood that very low absolute pressure readings of from 500 microns to 20 microns or less are necessary for efficient pouring of highly alloyed metals. I have also determined that by thus producing and holding extremely low pressure readings at the degassing chamber through which the stream of molten metal is conducted, I am able to produce very desirable results in that there is accomplished a greatly increased removal of harmful gases. Also, I am able to prevent the reoxidation and reabsorption of gases such as may occur when ladle degassed metal is repoured into ingot molds exposed to the open atmosphere.

I have further devised a method of vacuum casting a number of metal ingots in which molten metal is released to a series of ingot molds in predetermined successive time intervals and in which a vacuum pump apparatus moved from one sealing position to another on successive molds in a controlled sequence.

The nature of the invention and other objects and several features will be more apparent from the following description of preferred embodiments selected for pur-

poses of illustration and shown in the accompanying drawings, in which:

FIGURE 1 is a vertical cross sectional view of one simplified form of vacuum casting apparatus of the invention and indicates diagrammatically the operation of pouring molten metal while a vacuum is being exerted;

FIGURE 2 is an enlarged fragmentary view of the vacuum casting components and sealing means of FIGURE 1 including a heating device for inducing selective expansion of the sealing means;

FIGURE 3 is a vertical cross sectional view of another form of vacuum casting apparatus particularly suited for casting a number of ingots from one pouring ladle and also illustrating another form of expansion device;

FIGURE 4 is a fragmentary perspective view broken away at one point to illustrate more clearly the sealing means shown in FIGURE 3;

FIGURE 5 is a perspective view of the casting mold construction of FIGURE 3 and shown separated from the degassing chamber portion of the apparatus to indicate a special channel construction;

FIGURE 6 is a cross sectional view illustrating vacuum pump and control valve mechanism of the invention as employed at the left hand side of FIGURE 3;

FIGURE 7 is a perspective view illustrating the vacuum casting equipment combined with apparatus for carrying out a number of pourings from a single ladle member;

FIGURE 8 is a fragmentary plan view further illustrating the expandible sealing means employed in FIGURES 3 to 7 inclusive;

FIGURE 9 is a cross sectional view taken approximately on the line 5—5 of FIGURE 8;

FIGURE 10 is a fragmentary view illustrating a modified form of casting mold formed with an upstanding flange portion with which the sealing means of the invention may be associated;

FIGURE 10a is a fragmentary detail view of a portion of the mold structure shown in FIGURE 10 and illustrating sealing means in a position assumed before a vacuum is produced;

FIGURE 10b is another view similar to FIGURE 10a, but showing the position of a sealing member after a vacuum has been produced;

FIGURE 10c is a view similar to FIGURES 10a and 10b, but further illustrating the casting mold and sealing means under vacuum and expanded by heat resulting from a pouring operation;

FIGURE 11 is a fragmentary perspective view of casting mold means and another desirable arrangement of sealing means mounted thereon;

FIGURE 12 is an elevational view partly in cross section illustrating another modified casting mold means having the sealing means of the invention associated therewith;

FIGURE 13 is a cross sectional view illustrating vacuum casting apparatus of the invention;

FIGURE 14 is a plan view illustrating diagrammatically another type of vacuum pumping apparatus for use in teeming metal in successive ingot molds;

FIGURE 15 is a cross sectional view further illustrating the vacuum pumping apparatus of FIGURE 14 on a larger scale and indicating sealing components of the apparatus in a closed position;

FIGURE 16 is a diagrammatic view illustrating in graph form a time curve for ingot pouring intervals; and

FIGURE 17 is a cross section taken on the line 17—17 of FIGURE 13.

The method of sealing of the invention may be employed with various forms of casting components and may be designed to provide very low pressure. For example, FIGURES 1 and 2 illustrate a relatively small volume degassing chamber structure mounted on a casting mold, and a sealing body arranged externally of the line of junction of these members to provide for one type of vacuum

casting. FIGURES 3 to 9 illustrate a somewhat different arrangement in which the sealing body is protectively arranged around an expansion device to provide very low pressure micron readings for vacuum casting operations where a series of casting molds are used. FIGURES 10, 10a, 10b, 10c, 11, 12, 13, 14 and 15 illustrate still further modifications of the sealing means of the invention.

Considering first the form of invention illustrated in FIGURES 1 and 2, numeral 2 denotes an ingot casting mold 2 having an ingot cavity 4. One type of conventional mold now commonly used may have a cavity volume of approximately 16 cubic feet, for example. This mold member is preferably seated on a heavy flat bottom stool 6. At its upper side the ingot mold is formed with a generally flat but rough and non-uniform seat surface 8 which extends around the ingot cavity 4 to provide a support for a degassing chamber member generally indicated by the arrow 10. The degassing chamber and casting mold are sealed together by the sealing means of the invention as noted below. Conventional existing cast iron molds of the type used in the foundry can be economically used in the method of the invention.

In one suitable form the degassing chamber 10 includes an upper container section 10a, and a lower conduit section 10b. These sections are separated by a transverse wall 10e through the center of which is formed a pouring aperture 12 which is normally closed by a fusible closure cap 14 of aluminum or other suitable material. The cap 14 is secured by bolts 16 and 18. In the presence of hot metal discharged from transporting ladle 22, for example, shown at the upper side of FIGURE 1, the closure member 14 becomes fused and will then allow the hot metal to flow through the aperture 12 and down through the conduit section 10b to finally be received in the mold cavity 4.

A novel feature of the combination of degassing chamber section and mold member resides in providing the degassing chamber with a volume which is less than the volume of the mold. For example, with a mold cavity of 16 cubic feet, as noted above, I find I may employ a degassing chamber volume of approximately 5 cubic feet and I find that by thus employing a degassing chamber volume less than the volume of the mold cavity, I am enabled to obtain unexpectedly rapid pump-down to a degree such that micron readings as low as 200 microns in a time interval of 15 seconds may be obtained. This has not been accomplished in the art before in vacuum casting.

In the lower conduit section 10b is also supported an annular refractory "hot top" 19, which is necessary on all deoxidized steels.

I further construct the degassing chamber 10 with means for evacuating gases from the conduit section 10b as indicated in FIGURE 1. The evacuating means includes a passageway formed through the sidewall portion of the conduit section as shown and into which is tightly fitted a tubular member 26. Attached at some convenient point to the outer end of the tubular member 26 is a conventional vacuum pump unit which is not shown in the drawings.

When a casting operation is to be carried out, the degassing chamber is located on the relatively rough and non-uniform upper surface of the casting mold and these parts are sealed in accordance with the invention. In forming a seal a body of special sealing compound 30 is located externally around the junction of the degassing chamber 10, and the casting mold 2. This sealing compound is applied in a sufficiently fluid condition so that when placed in contact with the metal surfaces of the degassing chamber and a casting mold, it will adhere to the surfaces of the casting components, and in spite of the inequalities of the rough and uneven noted surface. After the compound has been applied, it is cured by heating. It will be understood that the sealing compound may be applied either before or after the degassing chamber is

placed on the mold surface 8. In ordinary working conditions the degassing chamber and casting mold under usual melt shop conditions may be at temperatures from 100° F. to 400° F., at which temperatures, for example, satisfactory curing will take place. The seal compound 30 cures to form an expansible solid body tenaciously secured to the metal parts in contact with it. Before pouring takes place, air is evacuated from the degassing chamber and casting mold to produce a desired vacuum. Normally I find that in this period before pouring takes place an absolute pressure of approximately 10 microns or less may be reached in about thirty seconds. Pressures as low as 10 microns and below are consistent with pressures attained by continuing evacuation of air for a period of approximately one minute or less. Speed of pump down is highly critical in successive pourings, especially in pouring from a single ladle into a series of prearranged molds since temperature losses in the molten metal in the pouring tend to occur and produce undesirable solidification of metal in the casting components of the pouring ladle. It is not uncommon with existing processes to have solidified metal left in the ladle after pour, or to have the nozzle and stopper rod freeze together if too much time is wasted and the temperature loss of the molten metal in the ladle is sufficiently great.

The release of pressure on the molten metal as it leaves the nozzle and enters the degassing chamber causes violent evolution of gases such as hydrogen, nitrogen and oxygen in the form of carbon monoxide. These gases are drawn off by the vacuum pump. At the same time the molten metal as it collects in the ingot mold is caused to continuously ebbulate and in the course of this action a further removal of gases takes place.

The percentage of gases in the molten metal may, find, be very significantly reduced in both of these ways, i.e., from the dispersed material and the collected material. Especially significant is a reduction in carbon content where the initial carbon content is low. This removal of carbon monoxide serves both as a deoxidation treatment for high carbon steels and a decarburization treatment and deoxidation treatment for low carbon content steel.

As the body of molten metal M collects in the casting mold 2, intense heat of the molten metal is conducted through the body portion of the casting mold at a much greater rate than occurs with respect to the degassing chamber section 10b. As a result the surface 8 of casting mold 2, undergoes in effect a thermal shock and expands differentially with respect to expansion of the degassing chamber section 10b.

However, in accordance with the method of the invention I find I may compensate for this differential expansion by utilizing a sealing material which is capable of deforming under stress to provide for a compensating expansion without splitting or separation taking place. Furthermore, the compensating expansion is accomplished with a compound whose unusual heat resistance characteristics enable it to withstand relatively high temperatures for a limited period of time, yet to thereafter decompose for ready removal from its mold and chamber surfaces.

As illustrative of temperatures to which the seal compound 30 may be exposed I may start, for example, with a mold which is at room temperature, or the mold may occur in a range of temperatures of from 150° F. to 400° F. The latter temperatures may occur as a result of an earlier used mold having cooled to these temperatures subsequent to removal of a steel ingot, or may be heated to these temperatures by any means such as a gas flame. The pouring interval may take anywhere from one to ten minutes to be completed and in this pouring interval temperatures from 100° F. up to 400° F. and possibly higher may occur, depending on the relative distance of the compound from the molten metal interface. The compound of the invention, for a short period after pouring, co-

ues to maintain itself in a vacuum-tight sealing con-  
ion and then starts to decompose as initially evidenced  
the smoking. The temperatures in the mold, after  
uring is completed, rise very quickly above 400° F. all  
way up to 1,500° F., and higher. At these tempera-  
res the sealing body 30 almost completely burns off  
leave a very thin powdery residue which can be readi-  
brushed away and replaced by new compound when  
sired.

Thus it will be observed that the compound exhibits  
veral desirable characteristics and performs a number of  
portant functions. First, there is a sealing with resis-  
tance to heat; secondly, there is a limited degree of de-  
formation to compensate for differential expansion of  
casting components during the short pouring inter-  
l; third, there is the ability to decompose and thus  
stitute a disposable sealing member which can be  
ickly replaced by a new sealing body without special  
aning operations.

The sealing compound 30, as noted above, may be of  
e class of compounds containing, in general, poly-  
oxide materials. Epoxy resins are prepared by the  
action of a dihydric phenol and epichlorohydrin in the  
esence of sufficient alkli to maintain the reaction mix-  
re substantially neutral.

The predominant constituent of the reaction product  
represented by the formula:



herein R represents a divalent aromatic hydrocarbon  
dical and n is an integer. By varying the ratio of  
ichlorohydrin to the dihydric phenol, compositions of  
varying molecular weight (varying n) may be obtained,  
a value of n decreasing as the quantity of epichlorohy-  
in is increased.

Considering for purposes of illustration the most widely  
ployed dihydric phenol, bis(4-hydroxy phenyl) di-  
ethyl methane (hereinafter termed Bisphenol A) the  
glycidyl ether has the formula:



here n of Formula 1 is zero. By employing a mole  
tio of epichlorohydrin to Bisphenol A of 10:1 the di-  
cidyl ether is produced in a fairly pure state. As the  
ole ratio is decreased the proportion of higher molecular  
ight polyethers increases. In general, mole ratios of  
1 to 10:1 give average molecular weights of about  
0 to 450. In practice it is found that though the size  
the major portion of the polyether molecules may be  
ntrolled, some small proportion of longer and shorter  
ight molecules will be present. In addition side reac-  
ns may occur with some formation of intermediates,  
t the quantity of these side products does not notice-  
ly influence the properties of the resin.

In preparing the sealing compound 30, I produce com-  
onent 1, the low molecular weight glycidyl ether by  
ing a dihydric phenol, bis(4-hydroxy phenyl) dimethyl  
ethane, having an average molecular weight of from  
0 to 450. With other dihydric phenols this range will  
ry slightly. Referring to Formula 1 the average mol-  
ule of the ether will contain between 1 and 1.5 R's  
romatic radicals) and n will vary from 0 to 1. The  
oxide equivalent (weight of resin in grams containing  
gram equivalent of epoxy) should be between about  
5 and 225. Assuming the resin chains to be substan-  
lly linear with an epoxy group terminating each end,  
en the epoxide equivalent is one-half the average mol-  
ular weight. The viscosity of the polyether will vary  
om 5,000 to 20,000 cps. as measured with a Brook-  
ld LVT-5X viscometer with No. 5 spindle at 6 r.p.m.

at 25° C. Many commercially available epoxy resins  
with suitable properties may be used. Among these are  
"Bakelite ERL-2774" and "Bakelite ERL-3794," "Epi-  
Rez 510," "Epon 820" and "Epon 828." "Bakelite" is  
5 the trade-mark of Union Carbide Corp.; "Epi-Rez" is the  
trade-mark of the Jones-Dabney Co., Div. of Devoe &  
Reynolds Co.; "Epon" is the trademark of the Shell Chem-  
ical Corp.

Component II is the reaction product of Component I  
10 with a glycol, for example, ethylene glycol. The ratio of  
epoxy to hydroxy can be varied from 1/0.5 to 1/2 with  
little effect on the finished compound. The reaction  
may be carried out by mixing the desired quantities  
15 of epoxy and ethylene glycol and heating to 150° to  
185° C. for one hour or until the mixture becomes  
homogeneous.

The product has a molecular weight of 385 to 485 and  
is believed to consist primarily of the product resulting  
from the reaction of one epoxide ring with an hydroxyl  
group of the glycol. Since Component I can be con-  
sidered to contain an average of two epoxy groups per  
molecule, it is quite certain that the primary condensation  
product resulting from such controlled conditions may be  
represented by the formula:



30 For convenience I shall refer to the condensation prod-  
uct as the 50% condensate of Component I with a glycol.

Component II lends flexibility to my resin composi-  
tion, but must be used in controlled amounts. I have  
found empirically that the ratio of Component I to Com-  
ponent II may vary from 20/80 to 12/88 with good  
35 results. When the quantity of Component II is more than  
88 parts, the resin after curing is gel-like and weak. When  
the amount of Component II is less than 80 parts, the  
composition cures to a brittle, easily cracked material.

40 The third Component III of my composition is a curing  
agent which acts to cross-link the epoxy compounds.  
The curing agent which I prefer to use is a mixture of a  
primary curing agent, pyromellitic dianhydride, and a sec-  
ondary curing agent selected from the group of organic  
45 acid anhydrides. The anhydride mixture is used in sto-  
chiometric quantities based on the amount of epoxy and  
hydroxyl groups present in the resin mixture. A slight  
excess, about 5%, is employed in the case of solid acid  
anhydrides to allow for uneven dispersion of the anhy-  
50 dride powders in the resin.

Anhydrides of dicarboxylic acids are well known in the  
art as curing agents and include phthalic anhydride,  
maleic anhydride, succinic anhydride, dodecenylsuccinic  
anhydride, and hexahydrophthalic anhydride.

55 Depending upon the particular anhydride curing agent  
used, the proportions of primary and secondary curing  
agents in Component III may be varied within certain  
well-defined limits. I have found that 2 to 15 parts of  
pyromellitic dianhydride and 43 to 17 parts of secondary  
60 anhydride for every 100 parts of resin give satisfactory  
sealing materials for high temperature uses.

65 The manner in which Component III is added to the  
epoxy composition will depend upon the particular anhy-  
drides in Component III. Phthalic anhydride must ordi-  
narily be passed with the resin through a colloid mill to  
get a good dispersion. Maleic anhydride, on the other  
hand, is sufficiently fine to be mixed in by hand.

70 When it is desired to shorten the curing time, various  
well-known cure accelerators may be added to the com-  
position. Among these are alphamethylbenzyl dimethyl  
amine, n-butyl amine, pyridine and n-methyl pyridine.  
These are used in catalytic amounts, from 0.5 to 3% of  
the weight of the resins in the composition.

In addition to the above basic ingredients it is advan-  
tageous to add various fillers to the composition to add

body, adjust viscosity, increase thermal conductivity and hence achieve more even cure and lower the coefficient of the thermal expansion. Among the fillers which can be used are atomized aluminum, iron, copper, aluminum oxide, silica powder, mica, and asbestos. Fibrous materials such as fine asbestos tend to bind the resin together and counteract differences in thermal expansion between the resin and the bonded metal. The quantity of filler may be varied from a few percent to three or four times the weight of the resin. The compounding manipulations are well-known to those skilled in the art.

The following examples illustrate the preparation of the compositions of my invention:

#### EXAMPLE I

A commercial epoxy resin, "Epi-Rez 510" with the following properties was employed as Component I:

|                           |        |
|---------------------------|--------|
| Viscosity, cps. at 25° C. | 12,000 |
| Specific gravity          | 1.15   |
| Color (Gardner scale)     | 3      |
| Epoxide equivalent        | 185    |
| Hydrolyzable Cl, percent  | 0.1    |

Component II is also a commercial epoxy resin, "Epi-Rez 507" which is the condensation product of Component I and ethylene glycol in the previously described ratios. It has the following properties:

|                           |      |
|---------------------------|------|
| Viscosity, cps. at 25° C. | 550  |
| Specific gravity          | 1.14 |
| Color (Gardner scale)     | 2    |
| Epoxide equivalent        | 385  |
| Hydrolyzable Cl, percent  | 0.15 |

Twelve parts of Component I was blended with 88 parts of Component II and 43 parts of phthalic anhydride and passed through a colloid mill to reduce the particle size of the phthalic anhydride to 0.025 mm. or less. Care must be maintained to keep the temperature below about 50° C. during passage through the mill. After cooling to room temperature 2.5 parts of pyromellitic dianhydride was added together with 55 parts of micronized silica, 35 parts of atomized aluminum, and 350 parts of short fiber asbestos. The mixture was thoroughly blended while maintaining the temperature of the mix below about 25° C. and 0.3 parts of pyridine were added to the mixture to act as a cure accelerator. The composition was applied to two steel rods about 2.5 cm. by 1.25 cm. by 30 cm. and the steel rods were pressed together end to end. These rods were heated to 205° C. for 15 minutes to cure the composition. The rods were then raised to 315° C., allowed to cool to room temperature and heated again to 345° C. The resin bond remained strong with no cracks or thermal decomposition noticeable.

As a further test of the ability of the composition of Example I to withstand high temperatures, a sample of the composition which had been cured at 205° C. for 15 minutes was placed in contact with a surface at 315° C. for a period of eight hours. There was no evidence of serious charring or decomposition, and the sample retained its normal compressibility.

#### EXAMPLE II

Component I was prepared in the manner described in U.S. Patent No. 2,682,515, column 6, under the heading "Polyether A."

Component II was prepared by adding 46.5 grams of ethylene glycol to 180 grams of Component I. The reaction mixture was maintained at 150° C. for one hour. Upon cooling there resulted a clear, low viscosity mono-functional-epoxy flexibilizer.

Sixteen parts of Component I was mixed with 84 parts of Component II and blended well at 25° C. To the mix was added 13.8 parts of pyromellitic dianhydride, 19.4 parts of maleic anhydride, 75 parts of micronized silica, 25 parts of atomized iron, and 150 parts of short fiber

asbestos. After mixing well a homogeneous blend of milk-like consistency was produced. To this was added 0.4 part of N-methyl pyridine to act as a cure accelerator.

The composition was spread on steel rods and baked for 20 minutes at 175° C. After carrying out the heating and cooling steps of Example I, the bond was found to retain its strength.

Though in the foregoing examples Component II was in each case a condensate of Component I and ethylene glycol, this need not be the case. Component II of Example I could have been substituted for Component II of Example II and vice versa. It is only necessary that Component II be approximately a 50% condensate of a glycol and a glycidyl polyether epoxy resin having a molecular weight between about 350 and 450, an epoxide equivalent of 175-225, between 1 and 1.5 aromatic radicals per polyether chain and a viscosity between 5,000 and 20,000 cps.

Also, though I have shown Component I to be made from Bisphenol A and epichlorohydrin for purposes of illustration, other dihydric phenols are suitable. These include resorcinol; 1,1-bis (4-hydroxyphenyl) ethane; 1,1-bis (d-hydroxyphenyl) propane; 1,1-bis (4-hydroxyphenyl) butane; 2,2-bis (4-hydroxyphenyl) butane and 1,1-bis (4-hydroxyphenyl) 2-methyl propane.

In thus providing a method of vacuum sealing in which the sealing body is expanded or otherwise deformed, may desire to control the expansion of the degassing chamber relative to the expansion of the casting mold in such a way as to further compensate for the differential expansion between these members. For example, in FIGURES 1 and 2, I have disclosed a heating coil 32 which is contained in a protective annular housing 34 mounted around the degassing chamber section 10b at a point immediately above the sealing body 30. Energizing the heating coil 32 by means of an electrical current operates to heat and expand the degassing chamber section 10b. This expansion may be controlled to compensate for the expansion of the casting mold 2, and by timing the electrical current with a rise in temperature in the casting mold 2, I may prevent or substantially reduce differential expansion.

It is pointed out that by thus controlling expansion of the degassing chamber, a lesser amount of flexing or deformation of the sealing compound is required to take place and, therefore, the operation of holding the several parts in substantially constant relationship to one another is made easier. This is illustrated in FIGURE 2, for example, by the broken line showings of the component parts 10b, 2 and 30 where the broken lines illustrate diagrammatically the controlled expansion of both the casting mold and the degassing chamber in very nearly the same degree.

In controlling the expansion of one casting component with respect to another, it will be apparent that compound of lesser yieldability characteristics may be employed for sealing purposes and it is intended that this method of compensatory expansion may be practiced with various sealing compounds which are capable of resisting thermal attack during the ingot pouring interval. It is also contemplated that mechanically induced expansion of one casting component relative to the other may be carried out by means of other devices such as hydraulically controlled expansion devices and the like.

In FIGURES 3 to 9 inclusive, I have illustrated another desirable form of method and apparatus for carrying out a degassing operation which is particularly suited to pouring a series of casting molds.

It will be understood that in steel foundries as presently equipped, there is provided a crane mechanism which is arranged to pick up a ladle filled with molten metal and carry the ladle to a pouring section of the melt shop where a series of casting molds are set up. Ordinarily, in typical operation there is an operator station which enables an operator to control the pouring of molten metal

to the casting molds one after another in rapid succession. Here it is very important to deal with a small volume and to employ a rapid pump down in providing for vacuum casting into a plurality of molds.

The apparatus illustrated in FIGURES 3 to 9 inclusive, concerned especially with this type of operation and as shown includes a platform P (FIGURE 7) along one side of which extends rails R, R1, on which is supported a mold truck T. Mounted in truck T are a series of casting molds C, C1, C2, C3.

The casting molds have secured thereto in sealed relationship respective degassing chamber units D, D1, D2 and D3. Located above the platform P is a travelling crane structure including an operator control unit O movable along elevated rails R2 and R3 on suitable pulleys. The crane structure further includes transversely supported rails R4 and R5 on which is received a travelling hoist H from which is suspended a pouring ladle L. Also supported on rail R3, and another rail R6, is a movable vacuum pump V and carriage V1.

In FIGURE 3, I have illustrated a pouring ladle and degassing chamber unit similar to those shown in FIGURE 7 and indicated on a somewhat larger scale. The structure of FIGURE 3 comprises the same type of casting mold already described in FIGURES 1 and 2, together with a suitable degassing chamber. In addition, however, FIGURE 3 illustrates a special compound containing a groove and a flexible sealing skirt component. The skirt is located at the bottom section of the degassing chamber as hereinafter described in greater detail.

Referring first to the ladle components of FIGURE 3, 1 comprises a conventional type pouring ladle which is fitted with a bottom discharge nozzle 60 having an adjustable stopper rod 62. Molten metal M1 is conducted from the ladle L1 into a degassing chamber 10' which is supported in sealed relationship on a casting mold 2'. Included in the degassing chamber structure is a bottom pouring ladle L2 which is fitted with a refractory lining 2'. A nozzle 22a provides an outlet for molten metal to leave the ladle L2 as suggested diagrammatically in FIGURE 3.

At its upper side the degassing chamber 10' is formed with a tubular section 11' having a flange 13' on which is received a ladle liner 18'. The latter member is formed with a flange 20b on which is mounted another flange portion 20a of the bottom pouring ladle L2. Numeral 0d indicates a sealing gasket. The ladle liner 18' is also fitted with a fusible aluminum or magnesium disc 26' maintained in sealed relationship with ladle liner 18' by flange member 24' and bolts as 24a and 24b. Suspended from the underside of the flange member 24' is a refractory spray shield 28' for confining the molten metal droplets in the line of travel indicated in FIGURE 3.

The degassing chamber 10' may be of any desired shape, for example, the outer housing portion shown in FIGURE 4 which terminates at its lower side in a bearing section 10c, having a box shape chosen to coincide with the rectilinear shape of the top of the casting mold 2' (FIGURE 5). The lower edge of bearing section 10c is supported on a top surface 8' of casting mold 2'.

In accordance with the invention, I combine with the degassing chamber a sealing member comprising a flexible wall or skirt 12' which is preferably constructed of metal and which is secured to the underside of the degassing chamber as best shown in FIGURE 3. The flexible wall 12' may, in the preferred form shown, be constructed with corrugations or pleats extending perpendicularly to the circumference of the skirt as is more clearly indicated in FIGURES 8 and 9, and also shown in FIGURE

This flexible skirt 12' has its lower edge embedded in a sealing compound 30' located in a groove 31' formed in the surface 8' of the mold 2'. The skirt extends all the way around the mold and constitutes a yieldable sealing wall which is especially designed to be extended per-

imetrically. It will be observed that the bearing section 10c occurs inside of this sealing skirt in a position to shield it from high temperatures occurring within the casting mold and degassing chamber when a pour is taking place.

It is further pointed out that the separated relationship of sealing wall 12' with respect to bearing section 10c provides a substantially enclosed space which in the presence of high vacuum, exerted by vacuum pumping means hereinafter described, constitutes an evacuated volume of high heat insulating character capable of retarding flow of heat from molten metal through the bearing section 10c towards the sealing wall 12'. Thus the sealing wall and also the portion of the sealing mass 30' occurring between the sealing wall 12' and the bearing section 10c, are protected by the evacuated volume of heat insulating character and there is avoided a flow of heat of sufficient intensity to effect the sealing capabilities of either the sealing wall 12' or the portion of the sealing mass 30' occurring between the sealing wall and the bearing section 10c during such periods as the sealing wall is being flexed as noted below.

In FIGURES 8 and 9, the flexible skirt 12' is shown on a somewhat larger scale and the broken line showings are intended to indicate diagrammatically changes in position of the groove, sealing body, and skirt occurring during differential expansion of the casting mold 2' during an ingot pouring interval.

As noted above the skirt 12' is preferably constructed of a flexible steel sheet which is corrugated along vertical lines of folding, as viewed in FIGURES 3 and 4. By reason of this corrugated construction and the type of steel used, the skirt is adapted to flex in two directions. It may flex in such a way that it increases in perimetric dimension with increase in perimeter of the casting mold groove 31'. Also, the bottom edge of the skirt may flex in or out relative to the top edge. Both of these changes are represented by the broken line showings in addition to the expansion which the compound itself undergoes.

I have found that under some conditions of differential thermal expansion, the combination of the compound, groove, and skirt provides optimum sealing results. It is believed that the corrugated skirt becomes extended with expansion of the mold groove. As the skirt expands it continues to maintain an anchored relationship in the bottom of the sealing compound in the groove while acting as a reinforcing medium for the sealing compound and materially reducing the stresses induced in the sealing compound itself.

It should be understood that as soon as a vacuum is established in the degassing chamber, atmospheric pressure tends to exert forces against the outer side of the skirt and that portion of the sealing compound which lies between the skirt and the outer edge of the groove. This occurs concurrently with the mold expanding and tending to stretch the sealing body at a time when the sealing is subjected to increasingly high temperatures. Thus there are various forces of deformation acting on the sealing body and the corrugated skirt exercises both a stabilizing and compensation action. Anchoring of the lower extremity of the skirt becomes especially important in view of the atmospheric pressure condition. In some cases the lower edge of the skirt may be supported at the bottom of the groove and in other cases I may desire to have the skirt occur in slightly spaced relation to the bottom of the groove.

For more clearly illustrating the positive sealing action between the bottom marginal portion of the skirt 12' which is of flexible steel and which may flex in two directions as stated, attention is called to FIGURES 10, 10a, 10b and 10c in which disclosures the skirt 12' is shown associated with a mold 2" formed with an upstanding flange having an outer face 12a providing an outwardly facing abutment against which the sealing compound or material 30a is positioned. The inner face of the skirt 12' is normally

positioned outwardly of the abutment and in sealing engagement with the sealing material 30a prior to the application of vacuum and the pouring operation, as shown in FIGURE 10a.

In FIGURE 10 there is illustrated the positioning of the skirt 12' when vacuum has been applied to the mold 2" at the initiation of the pouring operation. When vacuum is established in the degassing chamber, atmospheric pressure exerts force against the outer side of the flexible skirt and deflects the skirt inwardly so that pressure is applied by the inner bottom portion of the skirt to the sealing compound 30a to compress the same to insure and provide a positive seal against the outer face 122 of the abutment about the upper mold structure.

In FIGURE 10c there is illustrated in dotted lines at 2a the position of the mold 2" before it receives the molten metal. In the full line position the mold is shown after heating during the pouring operation and as indicated, the mold body 2" has been expanded outwardly so that the outer face 12a applies pressure to the sealing compound 30a against the adjacent inner face of the flexible skirt 12'. Thus as the pouring proceeds and as the temperature of the mold increases, an additional force is applied to the sealing compound due to the expansion of the mold and an ever increasing sealing effect is present as the pouring progresses and as the temperature of the mold increases. As a result of the foregoing, any disadvantages which might occur in the effectiveness of the sealing compound due to its curing by the heat of the mold is positively overcome by ever increasing pressure to the sealing compound by the continuous expansion of the mold structure.

The advantage of this new and novel concept is two-fold. In the first instance an effective seal is provided between the mold and the skirt instantly upon the application of vacuum due to the atmospheric pressure which positively deflects the flexible skirt inwardly against the sealing compound, and secondly, the sealing effect is gradually increased by the pressure applied by the mold structure during its expansion resulting from the absorption of heat from the molten metal being poured therein. Thus a gradual and ever increasing pressure is applied to the material forming the seal between the skirt and the outwardly facing abutment of the mold structure and while the sealing effect is continuous and gradually increased to provide maximum sealing, no damaging or excessive force is possible as the flexible skirt is capable of outward deflection should a condition occur in which maximum sealing effect and hardness of the sealing compound is approximated. In other words, every possible advantage occurs by the use of both inward and outward pressure against the sealing compound with the pressure on the compound gradually increasing during the pouring and in addition a safety factor is present which would prevent any hazards which might occur should the skirt be of such a character that it was incapable of necessary outward expansion. Obviously the operator of the invention is basically dependent upon the use of the depending, yieldable and extensible skirt portion, the use of which results in a positive initial sealing by atmospheric pressure against the fixed abutment 12a and a gradual continuous controlled increase in the sealing pressure between the flexible steel skirt and its applied pressure and the expanding fixed abutment during the pouring of the metal in the mold. This skirt portion is shown as formed of a plurality of wall portions disposed in angular relation to each other and angularly movable relative to each other.

In providing a vacuum with the sealing skirt arrangement described, I may also desire to add materials to the pour and I may wish to use special pumping equipment. At one side of the degassing chamber 10' is provided a sight port 40' having a removable high temperature optical glass 42' maintained in sealed relationship by means of a rubber gasket 44'. At an opposite side

of the degassing chamber 10' is a vacuum exhaust manifold 10d which is shown fragmentarily in FIGURE 3 and also indicated in FIGURE 6. The vacuum exhaust manifold communicates with a vacuum pump 78' and located between the manifold and the pump 78' is a valve mechanism including a pneumatically operated three-way high vacuum valve 70'.

The valve mechanism 70' includes an air release valve 72', a by-pass valve 74' and a main valve structure 90. The valve structure 90 has a valve shaft 92' supported in a shaft seal 98' to the lower end of which is fixed a closure disc 94' which is adapted to engage a valve seat 70a. This three-way valve mechanism is connected to the exhaust manifold in some convenient manner as, for example, by a flexible connection 50' and I may also employ a filter screen 76' located in a position to protect the valve mechanism from particles of molten metal and dirt in operation.

I may desire to add materials to the molten metal during the degassing operation in which case such addition may be made directly into the bottom pour ladle at the time of pouring, or I may provide an alloy addition mechanism as suggested at the right hand side of FIGURE 3. This alloy additions mechanism may include for example, a segmented barrel 32' mounted on a shaft 36a which is sealed at 36' in a suitable bearing member. Numeral 34' indicates a turning knob for rotating the segmented barrel at a point directly below a funnel 30. Material to be added to the pour is indicated at A in the container structure A' and passes through the funnel 30 down through a chute structure 30c. The container A is normally closed by a cover A''. The cover A'' is provided with a sealing means A'''.

In setting up the apparatus shown in FIGURE 3 preparatory to casting an ingot, I first provide a "hot top" 19' consisting of a body of refractory material which is positioned in the upper portion of the mold 2' as shown in FIGURE 3 and which is sealed by tamping steel wool into a narrow space provided between the inner surface of the mold 2' and the outer surface of the hot top 19'. The steel wool is denoted by the numeral 5'. It will be observed that the refractory body 19' comprises a substantial thickness of material which extends well below the top surface 8' of the casting mold 2', and thus the member 19' may function to provide heat insulation and to protectively shield the extreme upper surface of the casting mold 2' where the sealing compound 30' is located.

In applying the sealing compound 30', a quantity of the compound is provided in a liquid condition and introduced all around the casting mold groove 31' to substantially fill this space. While the compound is still in soft fluid condition, the sealing skirt 12' is located in the sealing material with the section 10c of the degassing chamber coming to rest on the top surface 8' of the casting mold. It will be observed that the lower edge of the sealing skirt 12' becomes thoroughly embedded in the compound and extends below the surface 8' of the mold for an appreciable distance. However, the hot top 19' projects well below the bottom of the groove 31' so that the heat insulating and protective effect above referred to is maintained all the way around the top of the casting. I have found that by thus employing a heat baffle and insulating medium in the manner described, I am enabled to retard the flow of heat from the molten metal into that part of the casting top where the groove and its compound occur. This is helpful in dealing with a compound which has limited resistance to thermal attack and insures that a premature decomposition of the sealing compound will not take place where a sealing mass of more limited heat resistance may be desired to be employed.

As earlier disclosed the preferred sealing compound is cured at temperatures of 100° F. to 400° F. and such temperatures may, in many cases, be present in a casting mold which has been used and allowed to cool. If the

old is not in this partly heated condition as a result of being cooled from standing for an extended period of time, then I may heat the mold. For example, I may employ a conventional gas burner which may be applied around the outer side of the mold or accelerator may be added to the compound. As soon as the compound is fully cured the apparatus is ready to receive molten metal.

In pouring a single ingot, the fusible aluminum or magnesium disc 26' may be maintained in sealed relation with ladle L2. In pouring a series of molds, however, the fusible disc 26' is attached to liner 18' by flange 24' and hinge bolts 24a in the manner already described. It will be observed that ladle L2, without the fusible disc may be inserted in a liner at any time and therefore may be transferred from mold to mold. This allows greater flexibility, fewer ladles L2, and less maintenance, skull removal, refractory repair, etc. Refractory lining 22' of ladle L2 may be heated, with a conventional gas burner, a dull red color before pour to prevent the formation of "skull," or solidification of metal in the lower section of ladle L2.

If additions to the pour is desired, carefully weighed alloy additions are placed in the alloy container and weighed and sealed by flange 30a and O ring 30'. Sight glass 42' is positioned over sealing ring 44'. Filter screen 7' is placed in valve inlet and sleeve 78' moved into position and secured. The assembly is now ready for operation and the vacuum pumps 50' are started.

The pumps 50', run continuously, blank-off at less than 30 microns against valve 70'. Three-way valve 70' is operated by a portable, three step, spring-loaded push button switch of conventional type and not shown in the drawings. The switch button is depressed to the first position and, normally open, air release valve 72', which is a 2" valve, is closed. The push button is then depressed a second position and, normally closed, by-pass valve 7', which is a 1" valve, is opened and air is removed from the mold cavity and manifold 10d until the pressure is reduced to below 200 millimeters. The push button is then depressed to a third position and valve disc 94', which is a 16" valve, is opened and the pressure quickly drops below 200 microns in a matter of seconds. If sufficient time is available, pressures of less than 1 micron are consistently obtained with degassing chambers and molds that have been used time after time without maintenance or machining.

By-pass valve 74' serves a dual purpose. To open a 1" disc against atmospheric pressure would require 000 lbs. of pressure. To open a 1" valve against atmospheric pressure requires 12 lbs. of pressure. By reducing the pressure differential across valve 94' to less than 2,000 microns, a small air cylinder may be employed for its operation. The by-pass valve also serves as a flow control valve for the blowers by allowing a limited flow of air to the pumps initially. A controlled flow of air through by-pass valve 74' minimizes the load on the blowers. I may, for example, employ a 25 hp. motor on a large Roots blower booster pump. This size motor will handle pressure differentials of 10 mm. across the blower whereas a pressure differential of 1 atmos. would require possibly a 150 hp. motor.

When the mold has been evacuated to less than 200 microns, metal M1 from ladle L1 is transferred from a melting furnace to a position so that nozzle 60 is directly above ladle L2. This may be a distance of approximately 10 inches. Stopper rod 62 is raised by an operator and metal M1 is discharged into preheated ladle L2. A liquid seal is quickly formed in the lower extremity of L2 due to its conical shape and small volume. The conical shape and small volume combine to do away with the necessity of a stopper rod. As the liquid seal is formed, metal proceeds through the nozzle 22a and melts fusible disc 26'. On entering the vacuum chamber, the stream separates to a shower of droplets in the manner earlier described.

The flaring of the stream at the nozzle may, for example, encompass an angle of approximately 90° to 120°. The design of the nozzle 22a is important in controlling the scatter of the metal stream by minimizing the tendency of certain viscous alloys to form a large bell-shaped icicle. This formation grows rapidly during pour until it welds to shield 28' and causes undue scatter and impingement of the stream on the hot top and mold wall.

As the stream falls through the degassing chamber, the scatter of droplets is minimized by collecting sleeve 28'. The sleeve 28' prevents the scatter of molten droplets from causing a buildup of solidified metal on the lower inside portions of the vacuum chamber, the hot top and the mold walls.

Impingement and erosion of the refractory hot top affects the cleanliness of the poured ingot and a buildup of droplets on the mold wall produces seams and scabs on the rolled and forged surfaces. Normally with collecting sleeve 28' in place I find that the surfaces of my vacuum cast ingots are far superior to air cast ingots.

During pour there is a further evolution of gas evolved from metal M1 in the mold. The combination of high vacuum, and cold rough mold surface promotes a further evolution of gas. As the metal level rises into hot top 19', steel wool 5' prevents metal from leaking up through between the hot top and the mold 2' and entering the hood.

When the metal level in the hot top 19' reaches to within an inch or two of the top, stopper 62 is lowered and the flow of metal from ladle L1 stopped. The balance of metal in L2 drains into the vacuum chamber and just fills the hot top. At the instant metal from L1 is stopped, valve control push button on switch 70' is released and main valve 94' and bypass valve 74' are closed and air release valve 72' is opened in timed sequence. Thus as the last metal leaves nozzle 22a air release valve 72' floods the vacuum chamber and manifold with air.

Without the air release valve it may be noted that the vacuum chamber and manifold would be flooded with air entering through nozzle 22a after the last metal is discharged from ladle L2. The blast of atmosphere through, for example, a  $\frac{5}{8}$ " or  $\frac{3}{4}$ " nozzle 22a, into a high vacuum chamber is sufficient to blow molten metal from the hot top and spray it around the entire vacuum chamber and manifold. As soon as the air release valve floods the vacuum chamber and manifold to atmospheric pressure, sight glass 42' is removed and tubular member 46' is inserted through sight port 40'.

After completion of the above procedure the manifold is removed. The mold and hood assembly are allowed to remain in position until such time as the poured metal in the mold is completely solidified. This may require an hour or more for a two to four ton ingot. During this period, heat from the solidifying metal raises the temperature of the mold to 1,000° F. to 1,500° F. and decomposes the sealing compound 30' to a powder. By the time the ingot is stripped from the mold, the compound is completely decomposed. After stripping, the mold groove 31' may be blown out or brushed lightly and is then ready to receive sealant again when cool enough.

Before pour, as earlier described, the mold is consistently evacuated down to 20 microns in about 30 seconds and if additional time is allowed pressures as low as one micron are attained as the refractory hot top is outgassed. It may be noted that an absolute pressure of .76 micron is one millionth of an atmosphere and during my pouring interval pressures of from 100 microns down to as low as 45 microns have frequently been observed. This is far below the 750 to 2,000 microns obtained by conventional vacuum casting operations.

The flexible sealing wall 12' and its arrangement relative to the degassing chamber 10' and casting mold 2' may be modified in various ways. For example, in FIGURE 11, I have illustrated a flexible sealing wall 12" which is

attached to a flange section 13" of a degassing chamber 15" by welding or other suitable means. The bottom of sealing member 12" is sealably engaged in a sealing mass 17" and also occurs in separated relationship to the inner bearing section of the degassing chamber 15" to provide an enclosed space. This enclosed space is capable of being evacuated to provide a heat insulating evacuated volume for protecting the sealing wall 12', as well as portions of the sealing mass between the sealing wall and the bearing section 10c from heat of molten metal delivered from a pouring ladle 19".

The sealing wall 12" may be a skirt of either rectangular, circular, or other desired form and is intended to be illustrative of any suitable metal or other material whose composition and shape in cooperation with a sealing mass and suitable heat insulating means will withstand relatively high temperatures for a short pouring interval while undergoing flexing action both inwardly and outwardly and maintaining a satisfactory sealing effect.

It may also be desired to utilize the flexible sealing wall and a sealing mass with other types of casting molds. For example, in FIGURE 12 there is illustrated a sealing wall 12g which is secured to a flange 13g of a degassing chamber 15g mounted on a stool 2g. The latter member constitutes a base for an upright mold component 4g which is located in separated relationship to the degassing chamber 15g to form an enclosed space 6g. The bottom of the sealing wall 12g is sealably embedded in a sealing mass 8g in a groove 9g in the stool 2g.

When molten metal from the ladle 10g is released into the mold 4g the air is pumped out of the degassing chamber through a conduit 16g, an evacuated volume 14g is provided and inward flexing of the sealing wall 12g occurs temporarily thereafter followed by outward flexing of the sealing wall as heat transmitted from the molten metal through the stool 2g causes this member to expand and extend the sealing wall and thus compressing the sealing mass 8g to provide a very tight seal.

In FIGURES 13, 14, 15 and 17, I have illustrated additional forms of mobile vacuum pump apparatus capable of being secured in an operative position with any one of a series of molds in a matter of a few seconds and just as rapidly disengaged. The apparatus of FIGURES 13, 14 and 15 differs from the movable pump means of FIGURES 3 to 7 above described in that high speed pump and connecting manifolds, together with control valves, are provided and the manifold means is supported on a travelling platform at a level corresponding very nearly to the height of the degassing outlet in mold and degassing chamber assemblies arranged in some suitable manner in a foundry pit. The high speed connecting manifolds also include mechanical clamping devices for very rapidly engaging the degassing chamber outlets.

This rapid change-over type of vacuum pumping apparatus constitutes one suitable means for carrying out a novel multiple ingot casting method in a predetermined time sequence which is related to the solidification characteristics of any particular molten metal which may be desired to be handled in a pouring ladle.

As earlier pointed out in the specification, trouble may develop with almost any kind of molten metal if time elapses in which the metal in the ladle has an opportunity to start to solidify or freeze before the pouring operations are completed. A chief cause of difficulty may be the tendency of the ladle stopper to stick or freeze in the ladle nozzle. This occurs where a portion of metal has just been released and the ladle stopper has been placed in a closed position. If too long an interval thereafter ensues the metal between the stopper and adjacent surfaces of the ladle nozzle starts to harden or solidify and freezing results.

I have found that this tendency varies with different types of molten metal which are poured and with some

types of molten metal the time interval may become critical. The solidification characteristics of any given molten mass contained in a ladle depends to some extent, for example, upon the temperature of the molten metal at the start of the pouring operation, as well as subsequent temperatures which may result from some cooling of the metal as it is moved from one pouring station to another.

Another factor controlling solidification characteristics of a molten metal is the composition of the molten metal. Thus a special alloy steel may start to solidify and cause freezing of a stopper in a ladle nozzle in a time limit of less than a minute, for example, after 40 to 50 seconds. A high grade carbon steel may, on the other hand, resist freezing or solidifying for a period of from 1 to 2 minutes. In the case of a low grade carbon steel, no difficulty may be experienced for an interval of from 2½ to 3 minutes and possibly longer depending upon temperature control employed.

Still another factor influencing the tendency of the ladle stopper to freeze is the nozzle pressure or head which is directly determined by the level or quantity of molten metal contained in the ladle above the nozzle aperture at any given time.

With these various limiting conditions in mind, I have devised a novel method of controlling the pouring of successive metal ingots and I refer to this novel method as "sequence vacuum casting" wherein the period occurring between closure of a ladle stopper in the ladle nozzle at the end of one pour, and opening of the ladle stopper at the beginning of a second pour, is controlled in accordance with the solidification characteristics of the metal to limit this period to a predetermined interval which is less than the freeze period of the particular metal being handled. This control is exercised at each ingot mold to provide for carrying out a series of successive steps in a predetermined timed sequence.

I have found that I am enabled to thus control sequential vacuum casting within permissible time limits for quick freezing metals by utilizing vacuum pumping apparatus capable of being applied and disengaged in a matter of a few seconds. In this way there is realized a change-over period of sufficiently shortened duration to avoid freezing of the stopper in the mold nozzle even when dealing with these very quick freezing molten metals.

In FIGURE 16, I have illustrated diagrammatically a typical sequence casting operation in which figure there is shown a time pressure strip recording for successive ingots poured from a heat of stainless steel in average pouring intervals of from 2½ to 3 minutes and wherein the change-over period from shifting the pours from one mold to another averages from 40 to 60 seconds.

With certain more critical materials, I find that I may carry out in sequence successive pump-down operations to pressures in a range of from 5000 microns down to as low as 25 microns in periods ranging anywhere from 10 to 40 seconds up to 10 to 300 seconds, and for certain quick freezing materials I may employ an optimum time interval in a range of as little as 10 to 45 seconds.

Considering in further detail the apparatus employed for carrying out this rapid sequential casting, reference is had to FIGURE 13. As shown therein numeral 102 denotes a casting mold having a degassing hood 104, together with an outlet 110 and a sealing skirt 106. Molten metal is furnished from a ladle 108 in the manner already described.

The outlet 110 is formed with a flanged portion 110a. A flexible tubular part 112a of a bellows member 112 is fitted over the end of outlet 110 in closely abutting relation to the flange 110a. The flexible part 112a is supported at an intermediate portion thereof around a rigid sleeve 112b within which is secured an end plate 110b designed to abut against the extremity of outlet 110 when the tubular part 112a is engaged as shown in FIGURE

3. Clamps as 112c and 112d may be employed to securely hold the flexible part 112a in place.

The bellows 112, at an opposite end thereof, is formed with a tubular part 112e tightly fitted around an outlet 14a of the member 114. Connected to the end plate 10b, by a universal connecting rod 115, is a reciprocating member 116. This member is internally threaded to receive a screw 117 turned by member 118 located externally of the housing 114 as shown.

By means of this arrangement the bellows member may be very quickly connected to the outlet 110 and adjacent surfaces are forced together by the reciprocating member 16 so that almost instant sealing may be realized as soon as the vacuum pumping apparatus has been located in a correct position relative to the outlet 110.

The bellows member 112 communicates with one side of the chamber 114 which serves as a dust collector and valve support. This member 114 in turn communicates with a valve body 120 as shown at the right hand side of FIGURE 13. Valve body 120 is formed with an opening 122 which is closed by a valve disc 124 when operated by an air cylinder 128. At the top of the member 114 is a release valve 130 which is controlled by an operator through a switch located at some convenient point near the apparatus.

The valve 120 communicates at 132 with a conduit and vacuum pump of the type indicated in FIGURE 7. The manifold 112, valve body 120, and vacuum pump referred to, are all movably supported in some convenient manner in the movable platform 134 as shown in FIGURE 13. The operation of the valve members 124 and 130 may be substantially the same as that of valves 90' and 72' described in connection with FIGURE 6, or these valves may be otherwise varied as desired. By means of these parts and the resulting rapid change-over, exceedingly short time intervals for pouring may be realized while still obtaining the benefit of vacuum treatment.

In FIGURES 14 and 15, I have illustrated a somewhat further modified form of vacuum pump apparatus in which a movable valve mechanism and connecting bellows are combined with a stationary vacuum pump and exhaust conduit. As noted in FIGURE 14, I provide an elongated stationary exhaust conduit member 150 which may consist of a cylindrical member located at one side of a casting mold pit. At spaced-apart intervals along the side of the conduit 150 are a number of cover members as 152, 154, 156 and 158 which can be removed to provide access to the interior of the conduit when desired. At one end of the manifold there may be provided a vacuum pump similar to the pump already described and adapted to evacuate gases from the conduit at all points thereof.

In accordance with the invention, I mount a valve supporting carriage 160 for slideable movement along the conduit 150. The carriage 160 is provided with U-shaped track members 162 and 164 adapted to engage at opposite sides of the conduit 150 as is better shown in FIGURE 5. Adjustably supported in the carriage in bearing members as 166 and 168 are retaining rods as 170, 172 which support in a laterally disposed position a valve structure 174 having a valve opening adapted to be located in position to communicate with any one of the openings closed by covers 152, 154, 156 and 158. The valve opening is indicated by numeral 176 and is adapted to be closed by reciprocable valve element 178 mounted on a shaft 180 in a bearing portion 182 of the valve body. The shaft 180 is operated by an air cylinder 184 so that the valve 178, when retracted, may take a position as shown in broken lines in FIGURE 15. At one side of the valve body 174 is a tubular connecting part 186 which is adapted to fit with a connecting part 188 in turn adapted to be connected to a degassing hood part 190 of a degassing chamber 191 as shown in FIGURE 14.

In operation the movable valve portion and its connecting parts can be moved from one station to another to connect with a desired inlet in the manifold 150 and similarly the portion 188 may be tightly connected to any one of the degassing hoods as suggested in FIGURE 14. This movable valve body may also be provided with release valves and by-pass valves of the sort already described and the operation of this valve may, in general, be the same as that earlier disclosed with reference to FIGURE 6.

Various other changes and modifications may be resorted to in keeping with the scope of the appended claims.

I claim:

- 15 1. In a method of sequence casting of metal ingots under vacuum in which vacuum pump apparatus is connected through a series of degassing chambers connected in sealed relation to a series of ingot molds in predetermined successive time intervals and portions of molten metal are periodically released from a removable pouring ladle, having a nozzle and an adjustable ladle stopper for opening and closing the nozzle, into a lower stationary pouring ladle which is connected to the degassing chamber, the steps which include applying a vacuum in one of the degassing chambers and its ingot mold, opening the ladle stopper after the movable ladle is positioned over the stationary ladle connected to the degassing chamber, pouring molten metal from the movable ladle into the stationary ladle and through the degassing chamber into the ingot mold until the mold and the stationary ladle are substantially full, closing the ladle stopper, continuing the application of vacuum, continuing the pouring of molten metal from the stationary ladle through the degassing chamber and into the mold to substantially fill the mold and as the pouring from the stationary ladle into the degassing chamber substantially ceases, discontinuing the application of vacuum and venting the degassing chamber to atmosphere, and thereafter sequentially repeating the above steps in connection with another degassing chamber and its ingot mold in timed relation to the temperature of the molten metal adjacent the ladle stopper so that the stopper is again opened to pour molten metal from the movable ladle to another stationary ladle before the molten metal adjacent the stopper has an opportunity to freeze, the time lapsed between each of the sequential openings of the ladle stopper being in the range of 10 to 300 seconds.
- 20 2. A method according to claim 1 in which the application of vacuum in the degassing chambers and ingot molds
- 25 3. In a method according to claim 1 in which the sequential openings of the ladle stopper provides absolute pressures in the range of 20 to 5000 microns.

#### References Cited by the Examiner

##### UNITED STATES PATENTS

- |    |           |         |                       |        |
|----|-----------|---------|-----------------------|--------|
| 55 | 448,945   | 3/1891  | Durfee et al. -----   | 22—73  |
|    | 1,320,770 | 11/1919 | Lougheed -----        | 266—34 |
|    | 2,190,209 | 2/1940  | Hozey -----           | 22—73  |
|    | 2,734,241 | 2/1956  | Southern et al. ----- | 22—73  |
| 60 | 2,970,351 | 2/1961  | Rice -----            | 22—79  |
|    | 2,996,772 | 8/1961  | Deacon -----          | 22—79  |
|    | 3,014,255 | 12/1961 | Bussard et al. -----  | 22—209 |
|    | 3,024,507 | 3/1962  | Gero -----            | 22—209 |
| 65 | 3,162,908 | 12/1964 | DeLuca -----          | 22—73  |
|    | 3,182,359 | 5/1965  | Gero -----            | 22—73  |
|    | 3,206,302 | 9/1965  | Finkl -----           | 75—49  |

##### FOREIGN PATENTS

- 70 227,391 5/1963 Austria.

J. SPENCER OVERHOLSER, Primary Examiner.

R. D. BALDWIN, Assistant Examiner.